

# United States Patent [19]

Simon-Vermot

[11] 3,738,101

[45] June 12, 1973

[54] TIMEPIECE ESCAPEMENT LEVER

[75] Inventor: Andre Simon-Vermot, 2400 Le Locle, Switzerland

[73] Assignee: Les Fabriques d'Assortiments Reunies, Garadet, Neuchatel, Switzerland

[22] Filed: Sept. 21, 1972

[21] Appl. No.: 290,828

Related U.S. Application Data

[63] Continuation-in-part of Ser. No. 52,093, July 2, 1970, Pat. No. 3,694,885.

[30] Foreign Application Priority Data

July 11, 1969 Switzerland..... 10608/69

[52] U.S. Cl. .... 58/116

[51] Int. Cl. .... G04b 15/00

[58] Field of Search ..... 58/116 R, 121 R, 58/122; 29/177, 178; 79/1.5

[56] References Cited

UNITED STATES PATENTS

|           |        |                   |            |
|-----------|--------|-------------------|------------|
| 3,335,562 | 8/1967 | Schneider .....   | 58/122     |
| 3,505,805 | 4/1970 | Cohen et al.....  | 58/116 R X |
| 3,511,340 | 5/1970 | Simon-Vermot..... | 58/121 A   |

Primary Examiner—Stephen J. Tomsky

Assistant Examiner—U. Weldon

Attorney—Dwight H. Smiley

[57] ABSTRACT

An escapement lever for a timepiece comprises a lever body including at one end a pair of divergent arms each carrying a pallet or pallet pin. The body is mounted on an arbor for oscillation with the pallets or pins cooperative with a toothed escapement wheel. The pallets or the pallet pins are coated with hard metal to increase wear, reduce friction and to facilitate lubrication.

12 Claims, 6 Drawing Figures



**FIG. 1****FIG. 4****FIG. 6****FIG. 2****FIG. 3****FIG. 5**

## TIMEPIECE ESCAPEMENT LEVER

## CROSS-REFERENCE TO RELATED APPLICATION

This application is a continuation-in-part of Application Ser. No. 52,093, filed July 2, 1970, now U.S. Pat. No. 3,694,885.

## BACKGROUND OF THE INVENTION

The usual escapement lever in a timepiece mechanism or movement comprises a metallic body secured to an arbor adapted for oscillation and having a pair of divergent arms each of which carries a pallet or a pin for cooperative engagement with the teeth of like radial projections of an escapement wheel. If pallets are employed, jewels, such as rubies, usually are mounted thereon to resist frictional wear but, in any event, it is difficult to maintain lubrication either of the jewels or the metal as in the case of pins.

## SUMMARY OF THE INVENTION

An escapement lever according to the present invention comprises a metal lever body, preferably having a safety pin at one end, the other end of which terminates in a pair of divergent arms respectively supporting a pallet or a pallet pin. The pallets or pins and, conveniently, the lever body, are coated with a hard metal such as electroless nickel, electroless chrome or a hard alloy such as cobalt-rhenium alloy, which has a low coefficient of friction and to which a lubricating oil of the type, for example, known as Synt-A-Lube, readily adheres. The escapement lever, including the safety pin and pallets may be stamped from a metal plate which then is coated with the hard metal or individually coated pallets or pins may be mounted on a lever body.

## BRIEF DESCRIPTION OF THE DRAWINGS

FIG. 1 is a plan view of an escapement lever comprising pallets integrally formed therewith;

FIG. 2 is a cross-sectional view taken on line 2-2 of FIG. 1;

FIG. 3 is a fragmentary plan view of a modified lever with individually supported pallets;

FIG. 4 is an enlarged fragmentary cross-sectional view taken on line 4-4 of FIG. 3;

FIG. 5 is a fragmentary plan view of an escapement lever having pallet pins, and

FIG. 6 is an enlarged fragmentary cross-sectional view taken on line 6-6 of FIG. 5.

## DETAILED DESCRIPTION OF THE INVENTION

Referring now to the drawing, specifically to FIG. 1, an escapement lever for a timepiece movement, in accordance with the present invention, comprises a lever 10 of elongated configuration having at one end a safety pin 12 and at the other end a pair of divergent arms 14, 14' respectively disposed on opposite sides of the longitudinal centerline of the lever, each carrying a pallet 16, 16'. The lever 10 is provided substantially on its longitudinal centerline with a bore 18 to receive an arbor 20 by which the lever is mounted for oscillation with respect to an escapement wheel, not shown.

According to the invention, the lever shown in FIG. 1 comprises a metal body which may be coated by a layer 24 of hard metal. The body may be blanked from any suitable metal such as brass, german silver, an alloy of one-third each of Cu, Ni and Mn, or steel, either before or after coating, and the hard metal preferably

comprises electroless nickel, an alloy of nickel and phosphorus containing from about 3.5 to 11.5 percent of phosphorus, the rest of the composition being constituted by nickel.

5 The lever body is subjected to a finishing operation to impart cold rolled properties thereto and provide a hardness of about 600° HV (hardness in the Vickers scale). If desired, the lever may be subjected to heat treatment to increase the hardness by precipitation of a phase. For the foregoing purposes, to increase the hardness up to about 800° HV, the lever may be subjected for about one hour at 600°C or for about 10 hours at 260°C.

After such heat treatment the coating has a coefficient of friction of about 0.2 and after this coating, for example, the area of the pallets 16, 16', has been lubricated, the coefficient friction is reduced to about 0.008. The electroless nickel is chemically deposited by dipping the lever body in a suitable bath to obtain a coating having a thickness of preferably less than 50  $\mu$ . Further, it is possible to coat the escapement lever by electroless nickel, e.g. by introducing the piece in a bath such as Enplate No. 415 or Niklad 792. The cold rolling effect produced by the finishing operation establishes a greater adhesion between the coating and the metal of the body.

Alternatively, the hard metal may comprise electroless chrome or a hard alloy such as a cobalt-rhenium alloy. A suitable bath may comprise Duralloy to form a coating of electroless chrome or a bath composed of 60 g/l of cobalt sulfate ( $\text{CoSO}_4 \cdot 7 \text{H}_2\text{O}$ ), 66 g/l of citric acid ( $\text{COOH} \text{CH}_2 \text{C}(\text{OH}) (\text{COOH}) \text{CH}_2 \text{COOH}$ , 10 to 30 g/l of perrhenate of potassium ( $\text{K-ReO}_4$ ) and about 10 g/l of perrhenate of ammonium ( $\text{NH}_4\text{ReO}_4$ ) as regenerator, to form a coating of an alloy of cobalt and rhenium. In the latter bath the density of current should be 2 to 12 Amp/dm<sup>2</sup>, the pH about 7.6 and the temperature about 55°C. Such coatings may be subjected to the finishing operations.

According to embodiments of the invention, the pallet members, whether pallets having substantial flat operative surfaces or pins having cylindrical surfaces, may be produced separately, at least their operative surfaces coated with the hard metal, and fixed to the lever. For example, as shown in FIGS. 3 and 4, a lever 10a may have arms 14a, 14a' divergent from an arbor 20a. The arms may have their extremities in the form of jaws defining slots 26, 26' within which are fitted pallets 16a, 16a', respectively, and which may be secured by any suitable bonding such as solder or adhesive. The pallets may comprise metal bodies 28 completely covered with a coating 30 of the hard metal or the coating may be limited to the operative surfaces of the pallets, that is those surfaces which operatively engage the escapement wheel.

Similarly, as shown in FIGS. 5 and 6, pins may be substituted for pallets. In this embodiment, a lever 10b has arms 14b, 14b' divergent from an arbor 20b and the extremities of the arms have bores 32, 32' respectively carrying pins 16b, 16b' which may comprise bodies 34 having a hard metal coating 36. Obviously, the pins may be suitably bonded in the bores. The coating of the individual pallet members, whether pallets or pins, may be effected in the same manner as previously described and the coatings have the same characteristics as previously described. Moreover, the pallet members may be

fixed to the levers prior to coating and thereafter both the lever and pallet members coated.

I claim:

1. A timepiece escapement lever comprising a lever body having a longitudinal centerline and an oscillator axis substantially intersecting said centerline, a pair of pallet members carried by said body on opposite sides of said centerline and having operative surfaces for cooperative engagement with an escapement wheel, coatings of hard metal on at least said operative surfaces of said pallet member, and said hard metal being from the group consisting of electroless nickel, electroless chrome and cobalt-rhenium alloy.
2. A lever according to claim 1 wherein said coating has a hardness of about 600° to 800° HV.
3. A lever according to claim 2 wherein said coating has a thickness of not more than 50  $\mu$ .
4. A lever according to claim 3 wherein said electroless nickel is an alloy of nickel and phosphorous, containing 3.5 to 11.5 percent phosphorus, the rest being nickel.

10

5. A lever according to claim 1 wherein said coating has a thickness of not more than 50  $\mu$ .

6. A lever according to claim 5 wherein said electroless nickel is an alloy of nickel and phosphorus, containing 3.5 to 11.5 phosphorus, the rest being nickel.

7. A lever according to claim 1 wherein said electroless nickel is an alloy of nickel and phosphorus, containing 3.5 to 11.5 percent phosphorus, the rest being nickel.

8. A lever according to claim 1 wherein said pallet members comprise pallets.

9. A lever according to claim 8 wherein said pallets are integral with said lever body.

10. A lever according to claim 9 wherein said pallets are at one end of said lever body, an integral safety pin, lever body and pallets.

11. A lever according to claim 10 wherein said coating has a hardness of about 600° to 800° HV and a thickness of not more than 50  $\mu$ , and comprises an alloy of 3.5 to 11.5 percent phosphorus with the rest being nickel.

12. A lever according to claim 1 wherein said pallet members are pins.

\* \* \* \* \*

25

30

35

40

45

50

55

60

65

UNITED STATES PATENT OFFICE  
CERTIFICATE OF CORRECTION

Patent No. 3,738,101 Dated June 12, 1973

Inventor(s) Andre Simon-Vermot

It is certified that error appears in the above-identified patent  
and that said Letters Patent are hereby corrected as shown below:

In the Foreign Application., Priority Data:

Change the Swiss number to 10607/69

Signed and sealed this 16th day of July 1974.

(SEAL)

Attest:

McCOY M. GIBSON, JR.  
Attesting Officer

C. MARSHALL DANN  
Commissioner of Patents